

March 5, 1963

H. HAYDN ET AL

3,080,230

PHOTOGRAPHIC STRATUM TRANSFER PROCESS AND ELEMENT THEREFOR

Filed Jan. 29, 1957



INVENTORS

*Hildegard Haydn*  
*Anita Von König*  
*Edith Weyde*  
BY  
*Connolly and Flutz*

ATTORNEYS

# United States Patent Office

3,080,230

Patented Mar. 5, 1963

1

3,080,230

## PHOTOGRAPHIC STRATUM TRANSFER PROCESS AND ELEMENT THEREFOR

Hildegard Haydn, Anita von König, and Edith Weyde,  
Leverkusen, Germany, assignors to Agfa Aktiengesell-  
schaft

Filed Jan. 29, 1957, Ser. No. 636,863

Claims priority, application Germany Feb. 18, 1956  
10 Claims. (Cl. 96—27)

The present invention relates to a process for the direct production of positives by means of silver halide emulsions which are developed by heat without application of any processing baths.

For the production of non-laterally reversed positive copies, it is already known to expose a silver bromide halide emulsion layer containing silver halide developing substances to the object to be reproduced and to heat said exposed material to temperatures of about 80–150° C. after it is brought into contact with a transfer layer. With this procedure, the developing substance, which is contained in the photographic silver halide emulsion layer and which has remained unused at the unexposed areas, is transferred to the transfer layer which is disposed in contact with the emulsion layer and which contains one or more substances which yield colored compounds with the said developing substance. Oxidizing agents and aromatic diazo and nitroso compounds are proposed by way of example as reactants in the positive layer.

It has now been found that direct positives are obtained in a simple manner if the silver halide developing substances which are used are those which so change the binding agent of the silver halide layer with the reduction of the exposed silver halide that it becomes infusible and unswellable, while the unmodified silver halide emulsion at the unexposed areas is used for building up the positive image by transferring the said unmodified silver halide emulsion to the transfer layer and reducing it in the transfer layer to a silver image. Such silver halide developing substances are referred to herein as tanning developers.

Suitable silver halide developing substances of this type are polyhydroxy compounds of benzene, naphthalene and diphenyl, which can be substituted in the nucleus by halogen atoms or alkyl, aralkyl, aryl or cycloalkyl groups, for example, pyrocatechol, hydroquinone, 2,3-dihydroxy naphthalene, 2,6-dihydroxy naphthalene, 3,4-dihydroxy diphenyl, 2,3-dihydroxy diphenyl, 1,2-dihydroxy-4-cyclohexyl benzene, 4-benzyl pyrocatechol and 4-cloro-pyrocatechol. With the application of heat, these developing substances not only reduce the exposed silver halide, but they also modify the gelatin, probably due to the formation of oxidation products, so that it becomes infusible and unswellable, while it remains unchanged at the unexposed places. This unmodified gelatin of the layer can now be brought during heat development or at a later stage into contact with a second layer which has the ability to adhere firmly to the unmodified gelatin so that, when the two layers are separated, portions of the gelatin are stripped from the negative layer. In this way, the non-laterally reversed positive of the copied original is obtained on the second layer, which is the so-called transfer layer, this positive being in the form of a gelatin relief which still contains silver halide and developing substance. If this gelatin relief on the transfer layer is now exposed to diffused light and again subjected to heat treatment, the record becomes deep black in color. A black coloring of the record can also be obtained by using an emulsion of appropriate composition or by adding suitable compounds to the positive layer. It is a particular advantage of the present process that

2

both the development process and the transfer process are effected only by heat and without any additional wet treatment.

The accompanying drawing is a flow sheet of the processes described herein.

5 Any silver halide emulsion can be used for the production of the negative layer, such as silver chloride, silver bromide, silver chlorobromide, and silver iodobromide emulsions. As binding agent, it is possible to use 10 those which are normally used in the photographic art and which are hardened by the action of heat by developer-oxidation products, such as for example, gelatin, polyvinyl alcohol, carboxymethyl cellulose and mixtures of these substances. The pH value of the emulsion is 15 preferably adjusted to about 3.5–6.5. In order to accelerate the initiation of the developing process, it is advisable to add non-tanning silver halide developing substances, such as p-methylamino phenol, p-amino phenol or their substitution products, to the hardening developer in amounts up to about 20% by weight as calculated on the tanning developer.

20 For stabilizing the developing substances, it is possible to add to the photographic layers substances which slowly split off sulphur dioxide or sulphurous acid and the 25 cleavage products of which do not cause either a hardening of the gelatin or any other undesirable influencing of the silver halide emulsion during storage. Examples of such substances are bisulphite compounds of such aldehydes or ketones as do not harden gelatin. Particularly 30 suitable for this purpose are aldehydes and ketones which have a relatively high boiling point, particularly a boiling point higher than 80° C. Such aldehydes are aromatic, araliphatic aldehydes, and heterocyclic aldehydes, such as benzaldehyde, terephthalaldehyde, cinnamaldehyde, 35 salicylaldehyde, furfural, whereas cycloaliphatic ketones, such as cyclopentanone and cyclohexanone, and araliphatic ketones, such as benzalacetone, and heterocyclic ketones, such as isatin, are the most suitable ketones. The acetone bisulphite compound would be less suitable, since 40 this substance only gives slight protection against oxidation of the developer because it has a comparatively strong tendency to decompose with volatilization of the acetone. Examples of substances which are particularly suitable are: Terephthalaldehyde bisulphite, cinnamaldehyde bisulphite, benzaldehyde bisulphite, salicylaldehyde bisulphite, cyclohexanone bisulphite, cyclopentanone bisulphite, and furfural bisulphite, these compounds being 45 preferably used in the form of their alkali-metal salts, such as their sodium, potassium, and lithium salts. The organic developing substances are preferably applied in 50 quantities of about 0.5–3 g. per 100 cc. of an ordinary silver halide emulsion, whereas the aforementioned stabilizers are preferably used in quantities of 0.2–2 parts per part by weight of organic developing substance.

55 In addition, it is important that compounds splitting off water should be added to the emulsion of the negative material or the transfer layer. Suitable additive compounds of this type are salts of inorganic or organic acids containing water of crystallization, such as for example, sodium citrate ( $C_6H_5O_7Na_3 \cdot 5H_2O$ ), sodium acetate ( $CH_3COONa \cdot 3H_2O$ ), calcium acetate

$(Ca(CH_3COO)_2 \cdot 2H_2O)$

60 trisodium phosphate ( $Na_3PO_4 \cdot 12H_2O$ ), sodium sulphate ( $Na_2SO_4$ ), and/or substances which ensure a high residual moisture content, such as, for example, glycol, glycerol, and sorbitol. These substances are preferably used in such amounts that the water content of the negative material amounts to 8–12, preferably 8–10 percent by weight. When these additives are used in the transfer layer, the moisture necessary in the development can

migrate during the processing from the transfer layer to the negative layer.

The negative layer can be arranged on any suitable layer support which is stable at the temperatures usually used for heat development, such as for example, paper, plastics, textile fabrics and metals. Between the support and the emulsion, it is advantageous to use an intermediate layer by which the holding strength of the emulsion layer is reduced so that the stripping of the unexposed gelatin is promoted. Particularly suitable for this intermediate layer are alcohol-soluble heat-resistant substances, such as ethyl cellulose, polyvinyl pyrrolidone, zein, polyethyl acrylate and polyvinyl acetate. Any suitable heat-resistant support can be used as transfer layer. The transfer layer can be any suitably coated or uncoated paper, or a plastic, fabric, or metal foil. With coated transfer papers the coating of the said paper can contain additives which split off water and also additives by which the transferred record is blackened, such as, for example, nitrogen-containing organic compounds as, for instance, N-diethyl aminoethanol, triethanolamine, tetramethyl ammonium hydroxide, pyridine, piperazine, hydrazine, or compounds containing sulphur, such as thioacetamide. These additives may be used in quantities of about 1-10 g. per 10 g. of binding agent, although other proportions are useful.

The production of the positive or the transfer process can either take place together with the developing process or at a later stage. Furthermore, several copies can be made from the negative, this taking place immediately after the first transfer or at different later stages. However, care should be taken that the negative is not exposed to light in the intervening period.

#### EXAMPLE 1

*Negative layer.*—20 g. of pyrocatechol, dissolved in a small amount of water, 10 g. of terephthalaldehyde bisulphite, 200 g. of sodium acetate containing water of crystallization ( $\text{CH}_2\text{COONa} \cdot 3\text{H}_2\text{O}$ ) and 0.05 g. of benztriazole are added to 1 liter of any desired silver halide emulsion. Other additives known in the emulsion art can also be used. The emulsion is cast on paper or another layer support and dried.

*Transfer layer.*—A 1% solution of acetyl cellulose acetobutyrate in acetone is cast on a layer support, such as, for example, paper, and then dried. It is advisable to add a plasticizer such as a phthalic acid ester, to the layer.

*Processing.*—After exposure to an image, the negative is brought into contact with the transfer layer. The negative and transfer layer are then subjected to a temperature of 90 to 150° C., preferably 110-120° C., for 5 to 30 seconds in a hot press. The transfer layer can be heated at a lower temperature. After separation, the gelatin of the unexposed areas adheres to the transfer layer. After subsequent exposure thereof with diffused light and after reheating, a deep black unreversed positive is obtained of the original image.

#### EXAMPLE 2

*Negative layer.*—20 g. of pyrocatechol and 2 g. of p-methylaminophenol sulfate in a small quantity of water, are added to 1 liter of any desired silver halide emulsion. This emulsion has added thereto 6 g. of cyclohexanone bisulphite, 180 g. of sodium acetate containing water of crystallization, and 0.05 g. of benztriazole or corresponding amounts of other stabilizers. This emulsion is cast on a support as in Example 1 and dried.

*Transfer layer.*—A 1% alcoholic solution of acetyl cellulose has 5 g. of piperazine per liter added thereto. The solution is cast on a support and dried.

*Processing.*—The processing takes place as in Example 1, but the after-treatment of the positive is superfluous since blackening of the transferred layer is effected by the piperazine.

#### EXAMPLE 3

*Negative layer.*—25 g. of 4-cyclohexyl pyrocatechol, dissolved in 30 cc. of dimethyl formamide, are added to one liter of any desired silver halide emulsion. 10 g. of terephthalaldehyde bisulphite, 225 g. of sodium acetate containing water of crystallization, 0.05 g. of benztriazole, and 0.03 g. of phenyl mercaptotetrazole are then added to the emulsion, which is then cast on a support as in Example 1 and dried.

*Transfer layer.*—A 2% solution of a copolymer of 30% acrylic acid and 70% of methyl methacrylate in dimethyl formamide is cast on a layer support and dried.

*Processing.*—As in Example 1.

#### EXAMPLE 4

*Negative layer.*—22 g. of monotertiary butyl pyrocatechol are introduced into 1 liter of silver chloride emulsion and then to the emulsion is added 200 g. of sodium acetate containing water of crystallization and 5.5 g. of cyclopentanone bisulphite. Stabilizers and other known additives such as wetting agents can be added.

*Transfer layer.*—A 3% solution of polyacrylonitrile in dimethyl formamide is cast on a layer support and dried.

*Processing.*—As in Example 1.

#### EXAMPLE 5

*Negative layer.*—20 g. of pyrocatechol, dissolved in a small quantity of water.

30 1 g. of p-methylaminophenolsulphate  
8 g. of salicylaldehyde bisulphite  
0.08 g. of benztriazole  
0.02 g. of phenyl mercapto tetrazole and  
35 15 cc. of glycerol

are added to each liter of a silver halide emulsion.

This emulsion is cast on a support as in Example 1 and dried.

*Transfer layer.*—3 cc. of N-diethyl aminoethanol are added to liter of a 3% alcoholic solution of a condensation product obtained from hexamethylene diamine adipate and caprolactam(epsilon-caprolactam).

*Processing.*—As in Example 2.

#### EXAMPLE 6

*Negative layer.*—The starting material is a silver halide emulsion in which 10 to 30% of the normal gelatin is replaced by one of lower constants, i.e. and a gelatin which has been partially degraded as, for instance, by heating an aqueous solution of gelatin at a temperature of 80° C. for several hours. Developer and additives can be those of Examples 2-5.

*Transfer layer.*—A fine mesh fabric such as silk gauze or plastic fabric is suitable as positive material. The fabric can also be coated with one of the aforementioned plastic solutions.

*Processing.*—As in Example 1.

#### EXAMPLE 7

60 *Negative layer.*—The starting material is a silver halide emulsion in which 15% of the gelatin is replaced by polyvinyl alcohol. The additives can be the same as in the preceding examples.

*Transfer layer.*—One of the layers described above is used as positive layer, and the processing then takes place accordingly.

#### EXAMPLE 8

*Negative layer.*—One of the emulsions described in the preceding examples is used as negative emulsion. It is cast on to a support which has been previously prepared beforehand with a weakly adhering layer. Suitable as the preparatory material are alcoholic plastic solutions, such as a 2% solution of ethyl cellulose in alcohol, these solutions being if necessary mixed with some gelatin.

75 *Transfer layer.*—One of the layers hereinbefore de-

scribed is used as positive and also an ordinary piece of writing paper.

*Processing*.—As in Example 1.

#### EXAMPLE 9

A silver chloride emulsion with the following additives per liter of emulsion is used for producing the negative layer:

20 g. of pyrocatechol, dissolved in a small amount of water,  
10 g. of terephthalaldehyde bisulphite,  
0.1 g. of nitrobenzimidazole, and also  
0.05 g. of mercaptobenzthiazole.

*Transfer layer*.—The paper is impregnated with a 10% sodium acetate solution and is then used as the transfer paper. On being heated, this paper gives off a certain amount of water which accelerates the reactions.

*Processing*.—As in Example 1.

#### EXAMPLE 10

##### *Negative layer*.—

20 g. of 2,3-dihydroxy naphthalene,  
5 g. of terephthalaldehyde bisulphite,  
0.05 g. of benztriazole,  
0.02 g. of mercaptobenzthiazole,  
10 g. of sodium acetate trihydrate ( $\text{CH}_3\text{COONa} \cdot 3\text{H}_2\text{O}$ ), and  
5 g. of sorbitol

are added to each liter of a silver chlorobromide or silver chloride emulsion.

This solution is cast onto a paper which has been treated beforehand with a 1% alcoholic solution of ethyl cellulose.

*Transfer layer*.—Any desired writing paper can be used.

*Processing*.—After exposure, the negative is brought into contact with the transfer layer. The negative and transfer layer are then passed between two heated rollers, in which they are subjected to a temperature of approximately 90 to 150° C. The two layers are then quickly pulled apart, only some of the unexposed negative layer remaining adhering to the positive (transfer) paper. The operation can be repeated 3 or 4 times in the same way. The thickness of the negative layer is of importance, since it is possible to produce more copies with a thicker coating of negative layer.

We claim:

1. A photographic material for preparing positive photographic images without the use of bodies of processing liquid, said material including a support and a light-sensitive tannable silver halide emulsion layer on the support, the emulsion layer containing an effective amount of a tanning developer, a non-tanning developer in an amount effective to accelerate the initiation of the development, and for every part by weight of developer about 0.2 to 2 parts by weight of a bisulphite of a compound selected from the group consisting of aldehydes and ketones that have a boiling point above 80° C. and that do not harden the emulsion.

2. A photographic material for preparing positive photographic images without the use of bodies of processing liquid, the said material including a support and a light-sensitive tannable silver halide emulsion layer on the support, the emulsion layer containing an effective amount of a tanning developer, a compound that evolves moisture at a temperature between 80 and 150° C. and in a concentration such that the water content of the emulsion is from 8 to 12%, and a bisulphite of a compound selected from the group consisting of aldehydes and ketones that have a boiling point above 80° C., the bisulphite being

present in a concentration between 0.2 and 2 parts by weight for each part by weight of the developer.

3. A process for the production of non-laterally-reversed positive photographic images without the use of bodies of processing liquid, which process comprises exposing to an original image a light-sensitive silver halide emulsion layer containing a tanning developer that causes the emulsion to be tanned in its photographically exposed areas when developing action takes place, and also containing, in an amount between 0.2 and 2 parts by weight per part by weight of the developer, a bisulphite of a compound of the group consisting of aldehydes and ketones that have a boiling point above 80° C. and that do not harden the emulsion layer, pressing the exposed emulsion layer against a transfer layer at a temperature between about 80 and 150° C., at least one of these two layers containing a moisture-evolving compound that provides sufficient water for the hot pressing to effect development and to cause undeveloped portions of the emulsion layer to adhere to the transfer layer, and thereafter separating the transfer layer from the emulsion layer so that the transfer layer removes the adherent portions of the emulsion layer and provides the desired photographic image.
4. A process as defined in claim 3 in which the moisture-evolving compound contains water of crystallization.
5. A process defined in claim 3 in which the moisture-evolving compound is hydrated sodium acetate.
6. A process defined in claim 3 in which the moisture is supplied by incorporating in one of the layers a moistening compound selected from the class consisting of glycol, glycerol and sorbitol.
7. The process of claim 3 in which the transferred portions of the emulsion are made darker in appearance.
8. The process of claim 3 in which the emulsion contains a non-tanning developer in addition to the tanning developer, and the transfer operation is conducted under conditions that cause the non-tanning developer to darken the transferred portions of the emulsion.
9. A process as defined in claim 3 in which the transfer layer contains a blackening agent that causes the blackening of the transferred portions of the emulsion.
10. A process defined in claim 9 in which the blackening agent is selected from the class consisting of N-diethylaminoethanol, triethanolamine, tetramethylammonium hydroxide, pyridine, piperazine, hydrazine, and thioacetamide.

#### References Cited in the file of this patent

##### UNITED STATES PATENTS

- 742,405 Eichengrün ----- Oct. 27, 1903  
1,954,325 Martinez ----- Apr. 10, 1934  
2,596,756 Yutzy et al. ----- May 13, 1952  
55 2,675,313 Yutzy et al. ----- Apr. 13, 1954  
2,716,059 Yutzy et al. ----- Aug. 23, 1955  
2,747,999 Yutzy et al. ----- May 29, 1956  
2,835,575 Cowden et al. ----- May 20, 1958  
2,865,745 Chan et al. ----- Dec. 23, 1958

##### FOREIGN PATENTS

- 60 2,971,840 Germany ----- Feb. 14, 1961  
392,938 Great Britain ----- May 26, 1933  
399,269 Great Britain ----- Oct. 5, 1933  
65 427,962 Great Britain ----- Apr. 29, 1935

##### OTHER REFERENCES

- Foster et al.: An Introduction to General Chemistry, 3rd, ed., Van Nostrand Co. (1947), pp. 104-5.  
Richardson et al.: General College Chemistry, 4th ed., 70 Henry Holt, 1947, p. 152.

UNITED STATES PATENT OFFICE  
CERTIFICATE OF CORRECTION

Patent No. 3,080,230

March 5, 1963

Hildegard Haydn et al.

It is hereby certified that error appears in the above numbered patent requiring correction and that the said Letters Patent should read as corrected below.

Column 1, line 43, for "naphthalene" read --- naphthalene ---; line 50, for "4-chloro-pyrocatechol" read --- 4-chloro-pyrocatechol ---; column 2, line 64, for "(Na<sub>3</sub>PO<sub>4</sub>·12H<sub>2</sub>O)" read --- (Na<sub>3</sub>PO<sub>4</sub>·12H<sub>2</sub>O) ---; line 65, for "(Na<sub>2</sub>SO<sub>4</sub>)" read --- (Na<sub>2</sub>SO<sub>4</sub>·10H<sub>2</sub>O) ---.

Signed and sealed this 1st day of October 1963.

(SEAL)

Attest:

ERNEST W. SWIDER

Attesting Officer

DAVID L. LADD

Commissioner of Patents